

## UNITED STATES PATENT OFFICE

1,992,110

## PROCESS OF CURING CONCRETE

Lester Wittenberg, New Rochelle, N. Y., assignor  
to The Barrett Company, New York, N. Y., a  
corporation of New Jersey

No Drawing. Application August 25, 1932,  
Serial No. 630,427

4 Claims. (Cl. 25—154)

This invention is directed to curing concrete, and more particularly, to the curing of concrete by suitably covering the surface of the wet concrete and maintaining the covering on the concrete until it is uniformly and evenly set.

It is well known that proper curing of concrete is important in order to obtain concrete without cracks or fissures and which will not become weak and brittle and therefore unsatisfactory for road surfacing, building, and other purposes. To accomplish proper curing of concrete is particularly difficult in the laying of roads and pavements because of the relatively large surface exposed to the air and sun which tend to dry the surface before uniform setting of the concrete has occurred.

It has been proposed to maintain the concrete covered with water by building earth dams thereacross at suitable intervals and filling the intervening spaces with water. This is quite costly; results in an unsightly appearance of the concrete road while under construction; and is not practical when the pavement is laid on a grade. Furthermore, the earth dams have a tendency to impair the concrete. It has been demonstrated that earth of alkaline nature occurring naturally in some localities may seriously impair the strength of the concrete.

Concrete has been covered with straw or pieces of burlap and these materials sprinkled at frequent intervals with water. Such curing procedure results in an unsightly appearance of the pavement construction and the application of straw and burlap to the concrete requires considerable manual labor. It is also exceedingly difficult to prevent the straw or pieces of burlap from being disturbed by the wind. Burlap or canvas has also been suspended on frames a short distance above the concrete. Such procedure is costly and the frames and covering are difficult to keep in place in windy weather. It has also been proposed to cover concrete with bitumen saturated roofing felt material that is substantially waterproof. Such procedure, in addition to requiring the use of the comparatively costly bitumen-saturated felt, renders it difficult to retain in the top portion of the concrete the necessary water to effect curing since the mixing water in the concrete tends to pass out through the bottom and insufficient water is retained in the top portion of the concrete to provide satisfactory curing.

I have discovered that concrete may be efficiently and economically cured by covering the surface thereof with felted fibrous material, such

as unsaturated roofing felt. The felt is preferably applied to the concrete substantially immediately after it is poured and readily absorbs water from the wet concrete and adheres thereto, no difficulty being experienced in its application or maintenance on the concrete even in windy weather. During the curing of the concrete, which may require as long as fourteen days, or longer, the felt is preferably wetted or sprinkled with water. The wetting may be repeated at intervals, the frequency depending on the humidity and temperature of the surrounding air, whether salt solution (e. g., calcium chloride) or water alone is used and like factors affecting the water retention of the felt. Two wettings with water per day will be sufficient to insure proper curing except under very dry atmospheric conditions, in which case water may be applied to the felt several times per day. Under very humid conditions, one wetting after application of the felt may suffice.

Felted fibrous material of open structure and high moisture-absorbing properties, such as made from rags, newsprint, wood pulp, bagasse, or other absorptive vegetable fibers in any desired proportions may be employed. It is important that the fibrous material be felted, and for best results, be composed of fibers that are highly water absorptive. Preferably, fibrous material having a porosity of not less than approximately 1.8 cc. of voids per gram is utilized.

To determine the cubic centimeters of voids per gram of felt, a small sample of felt (say 2" x 5") is dried for one hour at 100° C., cooled, desiccated, and thereafter weighed. It is then immersed in kerosene, maintained at a temperature of 25° C., for 18 hours. Thereafter, the sample is removed from the kerosene, drained in vertical position for 30 seconds, and again weighed. The difference in weight represents the kerosene absorbed. This difference in weight in grams, divided by the specific gravity of the kerosene, corresponds to the cubic centimeters of kerosene absorbed. This volume in cubic centimeters, divided by the original weight in grams, gives the voids in cubic centimeters per gram.

In the construction of cement concrete roads, the concrete may be mixed in the proper proportions in a mechanical mixer and deposited on the prepared sub-grade of the highway. The surface of the concrete is then levelled to the desired cross-section ordinarily by means of a mechanical finishing machine of any well-known type. As soon as the concrete has been levelled, dry unsaturated felt, felt paper, or felted mate-

rial of high moisture absorptive value is applied to completely cover the surface thereof. A felt weighing 28 pounds per 480 square feet and about  $\frac{1}{8}$  inch thick will result in satisfactory 5 curing. The felt material absorbs moisture from the concrete and instantly adheres thereto. The thickness of the felt may be varied to suit local climatic conditions, the length of time the covering will be maintained on the concrete, etc. For 10 colder climates preferably thicker felts are employed.

The felt may be made in varying widths best suited to each operation. It is preferably made 15 sufficiently wide so that it will cover the entire width of the concrete poured at one time thus eliminating the necessity of lapping two or more adjacent strips of felt. The felt rolls may be carried on trucks travelling on the erected side forms usually employed in the pouring of concrete. Such 20 a truck may be moved along continuously following the finishing machine, felt being unrolled from the truck as it moves and hence immediately protecting the freshly finished surface. If more than one strip of felt is necessary to cover 25 the width of concrete poured, two or more rolls may be mounted in staggered position on the truck and the felt therefrom unrolled and laid in somewhat overlapping parallel lanes.

The felt may be sprayed with a suitable hygroscopic salt solution, such as a calcium chloride solution, or sea water or the like, or dry calcium chloride or other hygroscopic salt may be placed on top of the felt, preferably after it is applied to the wet concrete. The calcium chloride or other hygroscopic salt will absorb water 30 from the air and may eliminate necessity for sprinkling the felt with water. Approximately one pound of calcium chloride or other hygroscopic salt may be added per square yard of felt.

In cases where the concrete is surface-treated, as for example with salts such as sodium silicate, the felt may be applied directly to the treated 40 concrete.

Among the numerous advantages possessed by 45 my invention over prior procedures of curing concrete may be mentioned the following:

(1) It is more economical to practice, particularly as compared with the use of burlap and saturated felt, and results in efficiently cured concrete. Burlap is comparatively expensive and 50 does not have the water absorptive properties of felt. As is well known, burlap is woven from jute, flax, hemp, or Manila fibers. Since it is a woven material, it is necessarily composed of twisted 55 yarn, which is much less absorbent than the fibrous constituents of roofing felt. In using burlap, excessive amounts of water must be applied to obtain penetration of the water through the burlap to the concrete.

(2) Burlap, when applied to wet concrete, due 60 to the fact that it is materially less absorptive than felt, will not immediately absorb moisture from the wet concrete, and in windy weather will be blown about and difficulty encountered in applying it. These difficulties are not present in the application of the dry felt of this invention.

(3) The application of dry felt is a cleaner operation than the application of burlap, straw, earth, etc., heretofore used and does not result 70 in an unsightly appearance of the roadway during construction. The dry felt can be removed from the road and disposed of at the end of the curing period much more economically than straw, earth, or similar material. When the concrete 75 is covered with bitumen saturated paper or felt,

there is a possibility that the mix-water in the concrete may flow out through the bottom of the concrete and insufficient water be retained in the concrete to provide satisfactory curing. The use of the felt of this invention will maintain the water on the surface of the concrete and provide a continuous additional supply of water to insure proper curing of the concrete.

(4) Dry felt is superior in its heat insulating properties to the materials used to protect green 10 concrete heretofore. This makes it possible to lay concrete earlier in the spring and later in the fall in localities where frost is encountered. In any locality the use of the felt of this invention 15 reduces the suddenness and extent of temperature changes to which the concrete is subjected with changes in weather conditions. When wet concrete is covered with wet felt and freezing weather sets in, I have found that the felt, freezing first, retains a layer of entrapped air between 20 it and the concrete. This layer of air acts as a heat insulator and protects the concrete for a considerable time against freezing. If the cold 25 is so extreme that in spite of the felt the concrete freezes, the effect of the freezing temperature is more uniformly distributed in the concrete and changes in the concrete occur more gradually. As a result, surface scaling of the concrete is substantially lessened or eliminated, and upon thawing, the concrete gains strength 30 more rapidly than would otherwise be the case.

(5) The felt, being light in color, i. e., of a light grayish hue, reflects heat, and at summer temperatures will maintain the concrete at a lower temperature than would be the case if dark materials, such as bitumen saturated felt of a blackish color or burlap of a dark brown color, were employed. Hence, evaporation of the water maintained in contact with the concrete is minimized.

(6) The felt, because of its felted fibrous characteristics adheres firmly to the surface of the concrete, which characteristic not only prevents the felt from being blown away by the wind as noted hereinbefore, but appears to cause the concrete on removal of the felt to have 45 a somewhat rough non-skid surface. The felt appears to absorb and remove some or all of the laitance on the surface of the concrete which may account for the non-skid surface produced. The removal of the laitance from the concrete, 50 I have found, avoids scaling and chipping of the concrete which may take place when the concrete is cured in accordance with prior procedures in which the laitance is permitted to remain on the concrete.

Heretofore, calcium chloride has been applied directly to the surface of the concrete. Application of calcium chloride directly to wet concrete, it has been found, results in scaling of 55 the concrete. In accordance with this invention, the application of calcium chloride to the felt covering over the wet concrete avoids scaling of the concrete and at the same time permits the utilization of the water absorbing and retaining properties of the salt.

Since certain changes may be made in carrying out the above process without departing from the scope of the invention, it is intended that all matter contained in the above description shall be interpreted as illustrative and not 70 in a limiting sense.

I claim:

1. The method of curing concrete, which consists in covering the surface of the wet concrete substantially immediately after it is poured with 75

light-colored water-absorbent sheet material composed of felted fibers, and maintaining said sheet material moist and in direct communication with the atmosphere during the curing.

5 2. The method of curing concrete, which consists in covering the surface of the wet concrete substantially immediately after it is poured with light-colored unsaturated roofing felt having not less than 1.8 c. c. of voids per gram of felt 10 and maintaining said felt moist and in direct communication with the atmosphere during the curing.

3. The method of curing concrete which comprises pouring the concrete and substantially immediately thereafter covering the surface of the wet concrete with light-colored water-absorbent felt having applied thereto a hygroscopic salt.

4. The method of curing concrete which comprises pouring the concrete and substantially immediately thereafter covering the surface of the wet concrete with light-colored water-absorbent felt saturated with calcium chloride.

LESTER WITTENBERG.